

# UNITED STATES PATENT OFFICE.

ALBERT C. HOLZAPFEL, OF NEW YORK, N. Y.

## PROCESS OF TREATING CONCRETE STRUCTURES TO WATERPROOF AND INSULATE THE SAME.

1,262,344.

Specification of Letters Patent.

Patented Apr. 9, 1918.

No Drawing.

Application filed December 19, 1917. Serial No. 207,909.

*To all whom it may concern:*

Be it known that I, ALBERT C. HOLZAPFEL, a subject of the King of Great Britain, residing at New York, in the county of New York and State of New York, have invented certain new and useful Improvements in Processes of Treating Concrete Structures to Waterproof and Insulate the Same, of which the following is a specification.

10 My invention relates to a process of treating concrete hulls of ships or vessels, to render the same water-proof and electrically insulated for the reception of copper or anti-fouling or other paints.

15 In accordance with the preferred embodiment of my process, the concrete hull, after the removal of the forms, is treated with a suitable cement wash, applied by a brush or trowel, in order to provide a smooth outer 20 surface. This smooth outer surface is allowed to thoroughly dry and harden. I then apply to this hardened surface a bituminous wash, which is preferably laid on by means of a large brush. This bituminous 25 wash preferably consists of 20 parts by weight of asphaltum, 20 parts by weight of coal tar pitch, and 60 parts by weight of coal tar spirit. This coating or wash is allowed to dry for about three to four hours.

30 After the bituminous wash is thoroughly dried, I next apply a coat of bituminous paint. This bituminous paint preferably comprises 15 parts by weight of asphaltum, 15 parts by weight of coal tar pitch, 15 parts by weight of heavy tar oil, 20 parts by weight of benzol or light tar oil, 3 parts by weight of linseed oil, 2 parts by weight of litharge, and 30 parts by weight of oxid of iron, or other suitable pigment.

40 The bituminous paint is used as a priming and will readily attach to the bituminous wash, which is first applied. This bituminous paint will serve as an insulator for copper paint or other anti-fouling paint, which 45 may be applied as a final coat.

I have found that the bituminous solution or wash will penetrate to a considerable depth into the structure of the concrete, thus water-proofing it to a high degree.

50 The bituminous paint will also further aid in water-proofing the concrete, and further serves as an insulator for a copper paint, and anti-fouling composition or other paint which it may be desired to subsequently ap-

ply to the surface, for protection against 55 fouling or to improve the appearance of the ship.

By the above means a reliable adhesion of the paint to the concrete can be assured.

It is obvious that either or both sides of 60 the concrete structure, may be treated or coated, in accordance with my process.

It is to be understood that the form of my invention herewith shown and described is to be taken as a preferred example of the 65 same, and that changes in the proportions of the several ingredients and order in which the steps are carried out may be varied without departing from the spirit of the invention or the scope of the subjoined claims. 70

Having thus described my invention, I claim:

1. The herein described process, which consists in applying a cement wash to the surface of a concrete structure for providing 75 a smooth surface, allowing the wash thus applied to harden, applying a bituminous wash to the hardened surface to water-proof the concrete structure and allowing the bituminous wash to thoroughly dry, applying a 80 bituminous insulating paint to the surface previously treated with the bituminous wash, and allowing the bituminous insulating paint to dry.

2. The herein described process, which 85 consists in applying a bituminous wash to a concrete structure to water-proof the concrete structure, said wash containing asphaltum, coal tar pitch, and coal tar spirit, allowing the bituminous wash to thoroughly 90 dry, applying a bituminous insulating paint to the surface previously treated with the bituminous wash, and allowing the bituminous insulating paint to dry.

3. The herein described process, which 95 consists in applying a bituminous wash to a concrete structure to water-proof the same, said bituminous wash comprising a bituminous material and coal tar spirit; allowing bituminous wash to dry; applying a bituminous insulating paint to the surface previously treated with the bituminous wash, said paint comprising a bituminous material, an oil, litharge, and oxid of iron; and allowing the bituminous insulating paint to 100 dry.

4. The herein described process, which consists in applying a bituminous wash to a

concrete structure to water-proof the same, said bituminous wash comprising asphaltum, coal tar pitch, and coal tar spirit; allowing the bituminous wash to dry; applying a 5 bituminous insulating paint to the surface previously treated with the bituminous wash, said paint comprising asphaltum, coal tar pitch, heavy tar oil, benzol, linseed oil,

litharge, and oxid of iron; and allowing the bituminous insulating paint to dry. 10

In testimony whereof I affix my signature in presence of two witnesses.

ALBERT C. HOLZAPFEL.

Witnesses:

RICHARD HOTTELEB,

EDWARD BOEHM.